

March 3, 1942.

K. MICHEL ET AL

2,275,085

GASKET MATERIAL

Filed June 19, 1941

Fig. 1.



Fig. 2.



Fig. 3.



Fig. 4.



Inventors  
Karl Michel  
Eugen Hutzenthaler

By

Foster & Codier  
Attorneys

## UNITED STATES PATENT OFFICE

2,275,085

## GASKET MATERIAL

Karl Michel, Stuttgart-Hofen, and Eugen  
Hutzenlaub, Stuttgart, GermanyApplication June 19, 1941, Serial No. 398,852  
In Germany September 13, 1939

3 Claims. (Cl. 28—1)

The present invention relates to flexible material for making gaskets and to gaskets made of the said material. The present invention also relates to resilient material to be laid or placed under a machine or other object to support it or to serve as a resilient support for something. The gasket forming material prepared according to the present invention is particularly useful in forming cylinder head gaskets for internal combustion engines, for example, such as are used in automobiles.

According to the present invention a woven fabric is prepared from narrow flat metal threads or strands and round, or approximately round, metallic yarn spun from metallic wool, as more fully appears hereinafter. The round or approximately round metallic wool yarns or strands are prepared from metallic wool, for example, steel wool, aluminum wool and copper wool. Round metallic yarn which is utilizable in the present invention is illustrated and described, for example, in the following U. S. A. Patents No. 1,012,030 granted December 19, 1911; No. 1,012,031 granted December 19, 1911; and No. 1,096,077 granted May 12, 1914. The term round as used in this description refers to the cross section of this yarn and the term round is intended to include round, approximately round, oval and intermediate shapes. The expressions "metallic wool strands" or "strands of metallic wool" are intended to include a bundle of the metallic wool in the form of a long mass of thread or cord-like shape, twisted or untwisted, and also compound yarns formed from two or more single yarns, threads, or cords twisted together.

The round metallic wool strands or yarns are used either as warp or weft in the woven fabric or gaskets of the present invention.

The narrow flat threads or strands in the woven fabric of the present invention are used either as warp or weft, and their thickness amounts to only a small fraction of the thickness or diameter of the round metallic wool strands or yarns. The flat strands may be flattened wire, or thin metal or metal foil cut into the form of narrow strips. The flat metal strands may be composed, for example, of iron, steel, aluminum or copper.

The round metallic wool strands and the flat narrow thin metallic strands are woven into the form of a fabric or cloth. Any kind of weaving can be used, for example plain weaving. However those kinds of weaving are preferred which produce a tight and strong woven material, for example twill weaving. The woven fabric formed

from these round and flat strands is smoother than it would be if it were woven wholly with round strands, particularly if the round strands are of large enough diameter to produce appreciable humps at the crossing points of the strands in weaving. Thus, according to the present invention, round metallic wool strands can be woven into the form of a comparatively flat or smooth fabric without the objection of humps or unevennesses produced by the crossing of these round strands in weaving.

The narrow flat metallic strands in the fabric and gaskets according to the present invention are not greater in width than  $\frac{1}{8}$  of an inch, and advantageously less than  $\frac{1}{16}$  of an inch. The thickness of the flat metallic strands in the fabric and gaskets according to the present invention is not greater than  $\frac{1}{120}$  of an inch and preferably less than  $\frac{1}{160}$  of an inch.

The round metallic wool strands may be of a diameter suitable for the use or uses to which the woven material or gasket is to be applied. However, we have found that when the round metallic wool strands have a thickness or diameter of  $\frac{1}{8}$  inch or less and the flat metallic strands have a thickness of  $\frac{1}{120}$  of an inch or less, irregularities or unevennesses in the thickness of the woven fabric are sufficiently avoided or reduced to render the woven fabric particularly suitable for use in forming gasket material and gaskets according to the present invention.

After the woven material is formed as above described it is impregnated with a binding medium which remains flexible after hardening or becoming hard, for example, rubber or an artificial rubber, or an artificial resin that does not become brittle at  $300^{\circ}$  F., and after such impregnation it is subjected to high pressure and heat, for example, between heated rolls. The impregnating medium may be incorporated in the woven fabric in a solution or liquid form, or even in a finely divided solid form, as long as it hardens, or solidifies, as a solid and binds together the strands of the fabric and fibers of the round strands together in compressed condition, upon the application of heat and pressure. The artificial resin used is of the type that hardens when heated.

The content of rubber, or of artificial rubber, or of artificial resin in the impregnated fabric is kept so low that these binding materials act practically only as pore fillers and as a means for holding the compressed fabric in compressed condition, and not as means for rendering the im-

pregnated material plastic or elastic from any elasticity of the binding agent per se, because the elasticity or resiliency of the finished material is to result alone, or in the main, from the strands of metallic wool. Therefore, the content of binder in the finished product is so chosen that it is present only in sufficient quantity to substantially wholly fill at least the pores of the fabric and to hold the pressed fabric in compressed condition after the pressure used in fabrication is released, whereby the pores of the fabric are practically wholly filled and the elasticity or resilience of the finished product is due practically wholly to the resiliency of the metallic wool strands under compression in the finished product. Obviously the compression in the above described operations of fabrication must not be carried so far as to destroy elastic resilience in the finished material, since the finished material must be able to be further compressed to some extent to be useful as gasket material.

Gaskets of desired shape and size may then be cut in any suitable manner from the material formed as above described.

Reference is now made to the drawing accompanying and forming part of this description. In the said drawing:

Figures 1 and 4 show in plan gasket material prepared according to the present invention.

Figure 2 is a section on the line *c-d* of Figure 1.

Figure 3 is a section on the line *a-b* of Figure 1.

In the embodiment illustrated in Figure 1 plain weaving is employed, while in the embodiment illustrated in Figure 4 twill weaving is employed. In the several figures the numeral 1 indicates the round strands of fine metallic wool which, after compression and binding in compressed condition, assume a more or less rectangular cross-section. In the several figures, the numeral 2 indicates the narrow strands of thin metal. The strands are preferably pushed close together in weaving and bound together with a binding agent of the type and in the manner described above.

We claim:

1. Gasket material comprising a fabric woven

from round strands of metallic wool and substantially flat strands of thin metal, the said fabric having its pores filled with a solid flexible binding agent, the amount of said binding agent being insufficient to impart an appreciable amount of elasticity from itself to the gasket material, and the said fabric being held in compressed resilient condition by the said binding agent but being able to be further compressed when used, the said gasket material possessing resiliency practically wholly due to the woven strands of metallic wool.

2. Gasket material comprising a fabric woven from round strands of metallic wool and substantially flat strands of thin metal, the thickness of said flat metal strands being only a small fraction of the thickness of said round metallic wool strands, the said fabric having its pores filled with a solid flexible binding agent, the amount of said binding agent being insufficient to impart an appreciable amount of elasticity from itself to the gasket material, and the said fabric being held in compressed resilient condition by the said binding agent but being able to be further compressed when used, the said gasket material possessing resiliency practically wholly due to the woven strands of metallic wool.

3. Gasket material comprising a fabric woven from round strands of metallic wool and substantially flat strands of thin metal, the said round strands being not greater than one-eighth inch in thickness and said flat strands being not more than one-eighth inch in width and not more than one one-hundred and twentieth of an inch in thickness, the said fabric having its pores filled with a solid flexible binding agent, the amount of said binding agent being insufficient to impart an appreciable amount of elasticity from itself to the gasket material, and the said fabric being held in compressed condition by the said binding agent but being able to be further compressed when used, the said gasket material possessing resiliency practically wholly due to the woven strands of metallic wool.

KARL MICHEL.  
EUGEN HUTZENLAUB.